

## UNITED STATES PATENT OFFICE.

EDWARD I. ALLISON, OF SAGINAW, MICHIGAN.

## COMPOSITION FOR PAVEMENTS.

SPECIFICATION forming part of Letters Patent No. 777,173, dated December 13, 1904.

Application filed December 28, 1903. Serial No. 186,883. (No specimens.)

*To all whom it may concern:*

Be it known that I, EDWARD I. ALLISON, a citizen of the United States, residing at Saginaw, in the county of Saginaw and State of Michigan, have invented certain new and useful Improvements in Composition for Pavements; and I do hereby declare the following to be a full, clear, and exact description of the invention, such as will enable others skilled in the art to which it appertains to make and use the same.

This invention is a composition of matter to be used for street-pavements and roof-coverings; and the improvement consists in a combination of certain ingredients in proportions stated and the equivalents thereof, as will be more fully set forth in the specification.

The objects of the invention are to provide a hard and durable material not easily abraded and capable of withstanding extreme cold and heat without cracking or flaking.

In practicing my invention I take of pulverized shale, such as is commonly procured from coal-mines, eighteen (18) parts and combine with it fifteen (15) parts of sand of medium fineness. This mixture is heated to about the temperature of boiling tar, and to it is added six (6) parts of stone-dust, or in lieu of the stone-dust, where an especially-strong mixture is required, Portland or similar cement. I take of pine-pitch ten (10) parts and mix with it from four (4) to six (6) parts of either pine-tar or coal-tar. This mixture is heated until it reaches the boiling-point and is then thoroughly mixed with the above-specified mixture of shale, sand, and stone-dust or cement.

Since shale from different localities absorbs different amounts of the melted pitch and tar, it is sometimes necessary to increase the above-specified quantity of the melted mixture that is to be added to the shale, sand, and stone-dust. Enough should be added in every case, however, to bring the entire mass to about the consistency of ordinary hot asphalt when laid for paving purposes.

It is found in practice that the pulverized shale imparts resilience and noiseless proper-

ties to the pavement and that the melted pine-pitch and tar forms a strong and elastic binding between the particles of sand. The binding qualities of the pitch are greatly increased and the cost of the pavement is reduced by mixing the pulverized shale and pitch, thus forming a material which fills the spaces between the particles of sand.

The office of the pine-tar or coal-tar mixed with the pine-pitch is to make a somewhat more fluid binding mixture than the pine-pitch alone.

The mixture of pine-pitch and pine-tar in the proportions specified forms a tougher and more durable binder than does the pine-pitch and coal-tar, although the latter mixture is cheaper and may be used in some cases, if desired.

Cement is added for the purpose of making the mixture set quicker and harder; but where the quickness of setting is not of great importance stone-dust may be substituted for the cement. By substituting in this mixture shale in the place of sand a somewhat coarser but softer mixture is obtained, which is found to be a very efficient paving material when laid between the concrete base and top dressing of an asphalt pavement, forming a slightly-elastic cushion beneath the top dressing.

While I have specified in the above mixture fifteen (15) parts of medium-fine sand, I prefer to produce the same result by using nine (9) parts of common river-sand and six (6) parts of fine sand, this mixture being equivalent for my purpose to the medium grade of fine sand, which is sometimes difficult to procure.

When the mixture is required to set quick but great hardness is not essential—as, for instance, in making sidewalk-blocks—I use plaster-of-paris in the above mixture in lieu of cement or stone-dust.

When used for pavements, the material is spread and rolled while hot, the process being practically the same as that now commonly used in laying ordinary asphalt pavements.

In the manufacture of roof-coverings I pre-

fer to roll the material while hot into sheets or layers, as is commonly done with composition roofing materials.

What I claim as my invention, and desire to 5 secure by Letters Patent, is as follows:

1. The herein-described composition consisting of shale, sand, stone-dust, pitch and tar, for the purposes set forth and substantially as described.
- 10 2. The herein-described composition con-

sisting of shale, stone-dust, pitch and tar, for the purposes set forth and substantially as described.

In testimony whereof I affix my signature in presence of two witnesses.

EDWARD T. ALLISON.

Witnesses:

W. I. CATHCART,  
A. A. EASTERLY.